

# United States Patent

Greiner et al.

[15] 3,705,495

[45] Dec. 12, 1972

[54] **FUEL SYSTEMS AND OXIDIZERS**

[72] Inventors: Leonard Greiner, Richmond, Va.;  
Welby G. Courtney, Dover, N.J.

[73] Assignee: Texaco Experiment Incorporated,  
Richmond, Va.

[22] Filed: Jan. 21, 1963

[21] Appl. No.: 253,523

[52] U.S. Cl. .... 60/214, 60/215, 60/216,  
60/219, 149/74, 149/109

[51] Int. Cl. .... C06d 5/08, C06d 5/10

[58] Field of Search .... 60/35.4, 214-216,  
60/219; 149/74, 75, 109; 23/152

[56] **References Cited**

UNITED STATES PATENTS

3,083,526 4/1963 Hudson ..... 60/35.4

2,504,119 4/1950 Frazer et al. .... 149/75  
2,968,539 1/1961 Wharton ..... 149/75  
2,975,045 3/1961 Perry et al. .... 149/75

Primary Examiner—Benjamin R. Padgett  
Attorney—Stowell & Stowell

## EXEMPLARY CLAIM

7. A method of producing thrust which comprises reacting in a combustion chamber an oxidizer comprising a liquid composition consisting essentially of from about 59 percent to about 77 percent by weight of perchloric acid, from 0 to about 15 percent by weight of  $\text{HNO}_3$  and the remainder water, the amount of water being sufficient to form dihydrated perchloric acid with at least about 95 percent of the perchloric acid and a fuel selected from the group consisting of light metals, metal hydrides, and mixtures thereof.

13 Claims, No Drawings

## FUEL SYSTEMS AND OXIDIZERS

This invention relates to improvements in fuel systems and fuel oxidizers for reaction motors.

It is an object of the present invention to provide fuel oxidizers and fuel systems which have good performance and are relatively safe to handle in that they do not produce toxic fumes, are very stable, and are relatively non-injurious to skin.

A further object is to provide fuel systems and fuel oxidizers which have good specific impulse and good density impulse and wherein the liquid component of the fuel system has a relatively high boiling point and a relatively low freezing point.

A further object is to provide a liquid-solid "hybrid" propellant system having particular utility and performance on boost-type missions but which may also be used for second-stage and sustainer missions. The propellant systems of the invention are of special utility in volume-limited rockets where the fuel density-impulse relationship is important.

These and other objects and advantages are provided in a liquid-solid propellant system comprising as an oxidizer dihydrated perchloric acid, and a fuel consisting predominantly of a light metal or a metal hydride and by an improved oxidizer for a light metal or a metal hydride comprising at least about 80 percent by weight of dihydrated perchloric acid.

It has been found that hybrid rocket propellants consisting of at least about 80 percent by weight of dihydrated perchloric acid as oxidizer and a fuel consisting predominantly of a light metal or a metal hydride provide very high performance on an integrated specific impulse and density basis, high safety, long storability and the capability of operation with the thrust of the reaction motor controlled over a wide thrust range by controlling the flow of liquid oxidizer to the fuel component of the hybrid system.

The following selected hybrid systems have been found to provide very satisfactory results:

| Solid (fuel)                                                                    | Liquid (oxidizer)                                                           |
|---------------------------------------------------------------------------------|-----------------------------------------------------------------------------|
| ZrH <sub>2</sub>                                                                | HClO <sub>4</sub> · 2H <sub>2</sub> O                                       |
| ZrH <sub>2</sub>                                                                | HClO <sub>4</sub> · 2H <sub>2</sub> O · HNO <sub>3</sub> · H <sub>2</sub> O |
| ZrH <sub>2</sub> · NH <sub>4</sub> ClO <sub>4</sub>                             | HClO <sub>4</sub> · 2H <sub>2</sub> O · HNO <sub>3</sub> · H <sub>2</sub> O |
| Zr+N <sub>2</sub> H <sub>5</sub> N <sub>3</sub>                                 | HClO <sub>4</sub> · 2H <sub>2</sub> O                                       |
| ZrH <sub>2</sub> · LiClO <sub>4</sub>                                           | HClO <sub>4</sub> · 2H <sub>2</sub> O                                       |
| ZrH <sub>2</sub> · Al                                                           | HClO <sub>4</sub> · 2H <sub>2</sub> O                                       |
| ZrH <sub>2</sub> · Al                                                           | HClO <sub>4</sub> · 2H <sub>2</sub> O · HNO <sub>3</sub> · H <sub>2</sub> O |
| Al-N <sub>2</sub> H <sub>5</sub> N <sub>3</sub>                                 | HClO <sub>4</sub> · 2H <sub>2</sub> O                                       |
| Al-N <sub>2</sub> H <sub>5</sub> N <sub>3</sub> · N <sub>2</sub> H <sub>4</sub> | HClO <sub>4</sub> · 2H <sub>2</sub> O                                       |
| AlH <sub>3</sub>                                                                | HClO <sub>4</sub> · 2H <sub>2</sub> O                                       |
| Mg(AlH <sub>4</sub> ) <sub>2</sub>                                              | HClO <sub>4</sub> · 2H <sub>2</sub> O                                       |
| (AlH <sub>3</sub> ) <sub>2</sub> N <sub>2</sub> H <sub>4</sub>                  | HClO <sub>4</sub> · 2H <sub>2</sub> O                                       |
| MgH <sub>2</sub>                                                                | HClO <sub>4</sub> · 2H <sub>2</sub> O                                       |
| MgH <sub>2</sub>                                                                | HClO <sub>4</sub> · 2H <sub>2</sub> O · HNO <sub>3</sub> · H <sub>2</sub> O |
| TiH <sub>2</sub>                                                                | HClO <sub>4</sub> · 2H <sub>2</sub> O                                       |
| TiH <sub>2</sub>                                                                | HClO <sub>4</sub> · 2H <sub>2</sub> O · HNO <sub>3</sub> · H <sub>2</sub> O |

Table I shows calculated performance data including the specific impulse for two illustrative ratios of reactants in the propellant system ZrH<sub>2</sub> — HClO<sub>4</sub> · 2H<sub>2</sub>O.

TABLE I

| Ingredients:                                                  | moles  | g/100g | moles  | g/100g |
|---------------------------------------------------------------|--------|--------|--------|--------|
| ZrH <sub>2</sub>                                              | 3.0000 | 67.204 | 4.2000 | 74.152 |
| HClO <sub>4</sub> · 2H <sub>2</sub> O                         | 1.0000 | 32.796 | 1.0000 | 25.848 |
| Computed Density, g/cc                                        |        | 3.211  |        | 3.530  |
| Performance:                                                  |        |        |        |        |
| Shifting I <sub>sp</sub> , sec                                | 203.2  |        | 148.5  |        |
| Shifting Volumetric I <sub>sp</sub> , lb-sec/in. <sup>3</sup> | 23.6   |        | 18.9   |        |

| Thermodynamic Characteristics:  | Chamber | Exhaust | Chamber | Exhaust |
|---------------------------------|---------|---------|---------|---------|
| Temperature, °K                 | 4212.0  | 2961.1  | 3353.8  | 2425.8  |
| Moles of Gas, moles/100g        | 1.683   | 1.5475  | 1.5366  | 1.5128  |
| Combustion Products, moles/100g |         |         |         |         |
| Gaseous Atoms                   |         |         |         |         |
| H                               | 0.3630  | 0.1884  | 0.0696  | 0.0247  |
| O                               | 0.0008  | 0.0000  | 0.0000  | 0.0000  |
| Cl                              | 0.0397  | 0.0231  | 0.0000  | 0.0000  |
| Zr                              | 0.0001  | 0.0000  | 0.1276  | 0.1281  |
| Gaseous Molecules               |         |         |         |         |
| H <sub>2</sub>                  | 1.0298  | 1.1159  | 1.2335  | 1.2563  |
| H <sub>2</sub> O                | 0.0179  | 0.0056  | 0.0000  | 0.0000  |
| OH                              | 0.0040  | 0.0003  | 0.0000  | 0.0000  |
| HCl                             | 0.1804  | 0.2112  | 0.0009  | 0.0000  |
| ZrO                             | 0.0026  | 0.0000  | 0.0108  | 0.0089  |
| ZrCl <sub>2</sub>               | 0.0099  | 0.0030  | 0.0942  | 0.0947  |
| Liquid and Solid Molecules      |         |         |         |         |
| ZrO <sub>2</sub> (1)            | 0.7080  | 0.7178  | 0.5627  | 0.0000  |
| ZrO <sub>2</sub> (s)            | 0.0000  | 0.0000  | 0.0000  | 0.5636  |

20 Table II shows calculated performance data including the specific impulse for an illustrative ratio of reactants in the propellant system ZrH<sub>2</sub> — NH<sub>4</sub>ClO<sub>4</sub> — HClO<sub>4</sub> · 2H<sub>2</sub>O — HNO<sub>3</sub> — H<sub>2</sub>O.

TABLE II

| Ingredients:                                                  | moles   | g/100g  |
|---------------------------------------------------------------|---------|---------|
| ZrH <sub>2</sub>                                              | 1.0189  | 72.092  |
| NH <sub>4</sub> ClO <sub>4</sub>                              | 0.04255 | 3.794   |
| HClO <sub>4</sub> · 2H <sub>2</sub> O                         | 0.26930 | 20.310  |
| HNO <sub>3</sub>                                              | 0.05302 | 2.536   |
| H <sub>2</sub> O                                              | 0.09274 | 1.268   |
| Computed Density, g/cc                                        |         | 3.156   |
| Performance:                                                  |         |         |
| Shifting I <sub>sp</sub> , sec                                |         | 193     |
| Shifting Volumetric I <sub>sp</sub> , lb-sec/in. <sup>3</sup> |         | 25.5    |
| Thermodynamic Characteristics:                                | Chamber | Exhaust |
| Temperature, °K                                               | 4718    | 3337    |
| Moles of Gas, moles/100g                                      | 1.7128  | 1.6906  |
| Combustion Products, moles/100g                               |         |         |
| Gaseous Atoms                                                 |         |         |
| H                                                             | 0.2128  | 0.1727  |
| Cl                                                            | 0.0191  | 0.0187  |
| O                                                             | 0.0005  | 0.0001  |
| Gaseous Molecules                                             |         |         |
| HCl                                                           | 0.1632  | 0.1930  |
| H <sub>2</sub>                                                | 1.2001  | 1.2322  |
| ZrCl <sub>2</sub>                                             | 0.0270  | 0.0125  |
| H <sub>2</sub> O                                              | 0.0491  | 0.0240  |
| OH                                                            | 0.0046  | 0.0009  |
| N <sub>2</sub>                                                | 0.0363  | 0.0363  |
| Liquid and Solid Molecules                                    |         |         |
| ZrO <sub>2</sub> (1)                                          | 0.7463  | 0.0000  |
| ZrO <sub>2</sub> (s)                                          | 0.0000  | 0.7608  |

55 Table III shows calculated performance data for an illustrative ratio of reactants in the propellant system Zr — N<sub>2</sub>H<sub>5</sub>N<sub>3</sub> — HClO<sub>4</sub> · 2H<sub>2</sub>O.

TABLE III

| Ingredients:                                 | moles   | g/100g  |
|----------------------------------------------|---------|---------|
| Zr                                           | 1       | 43.2    |
| N <sub>2</sub> H <sub>5</sub> N <sub>3</sub> | 1       | 35.4    |
| HClO <sub>4</sub> · 2H <sub>2</sub> O        | 0.3333  | 21.5    |
| Computed Density, lb/in. <sup>3</sup>        |         | 0.08079 |
| Computed Density, g/cc                       |         | 2.236   |
| Performance:                                 |         |         |
| Frozen Specific Impulse, sec                 |         | 233.5   |
| Thermodynamic Characteristics:               | Chamber |         |
| Temperature, °K                              | 4212.0  | 2961.1  |
| Moles of Gas, moles/100g                     | 1.683   | 1.5475  |
| Combustion Products, moles/100g              |         |         |
| Gaseous Atoms                                |         |         |
| H                                            | 0.3630  | 0.1884  |
| Cl                                           | 0.0008  | 0.0000  |
| O                                            | 0.0397  | 0.0231  |
| Zr                                           | 0.0001  | 0.0000  |
| Gaseous Molecules                            |         |         |
| H <sub>2</sub>                               | 1.0298  | 1.1159  |
| H <sub>2</sub> O                             | 0.0179  | 0.0056  |
| OH                                           | 0.0040  | 0.0003  |
| HCl                                          | 0.1804  | 0.2112  |
| ZrO                                          | 0.0026  | 0.0000  |
| ZrCl <sub>2</sub>                            | 0.0099  | 0.0030  |
| Liquid and Solid Molecules                   |         |         |
| ZrO <sub>2</sub> (1)                         | 0.7080  | 0.7178  |
| ZrO <sub>2</sub> (s)                         | 0.0000  | 0.0000  |

|                                 |        |
|---------------------------------|--------|
| Temperature, °K                 | 3579   |
| Moles of Gas, moles/100g        | 3.9223 |
| Combustion Products, moles/100g |        |
| Gaseous Atoms                   |        |
| H                               | 0.1731 |
| Cl                              | 0.0118 |
| Gaseous Molecules               |        |
| H <sub>2</sub>                  | 1.4122 |
| HCl                             | 0.1452 |
| N <sub>2</sub>                  | 1.1800 |
| Condensed Phases                |        |
| ZrO <sub>2</sub>                | 0.4720 |

Table IV shows calculated performance data for three illustrative ratios of reactants in the propellant system Al — N<sub>2</sub>H<sub>5</sub>N<sub>3</sub> — HClO<sub>4</sub> · 2H<sub>2</sub>O.

TABLE IV

| Ingredients:                                 | moles   | g/100g  | moles   | g/100g  | moles   | g/100g |
|----------------------------------------------|---------|---------|---------|---------|---------|--------|
| Al                                           | 1       | 19.615  | 1       | 15.842  | 1       | 11.310 |
| N <sub>2</sub> H <sub>5</sub> N <sub>3</sub> | 1       | 54.584  | 1       | 44.085  | 1       | 31.472 |
| HClO <sub>4</sub> · 2H <sub>2</sub> O        | 0.26    | 25.801  | 0.5     | 40.073  | 1       | 57.218 |
| Computed Density, lb/in. <sup>3</sup>        | 0.05874 |         | 0.05930 |         | 0.05999 |        |
| Computed Density, g/cc                       | 1.6258  |         | 1.6413  |         | 1.6604  |        |
| Performance: Frozen I <sub>p</sub> , sec     | 273.1   |         | 266.1   |         | 249.4   |        |
| Thermodynamic Characteristics:               |         | Chamber | Chamber | Chamber |         |        |
| Temperature, °K                              | 3312    | 3391    | 3260    |         |         |        |
| Moles of Gas, moles/100g                     | 4.2981  | 3.9172  | 3.5343  |         |         |        |
| Combustion Products, moles/100g              |         |         |         |         |         |        |
| Gaseous Atoms                                |         |         |         |         |         |        |
| Al                                           | 0.0099  | 0.0002  | 0.0000  |         |         |        |
| Cl                                           | 0.0080  | 0.0187  | 0.0437  |         |         |        |
| O                                            | 0.0001  | 0.0024  | 0.0126  |         |         |        |
| H                                            | 0.1357  | 0.1181  | 0.0329  |         |         |        |
| Gaseous Molecules                            |         |         |         |         |         |        |
| O <sub>2</sub>                               | 0.0000  | 0.0006  | 0.0402  |         |         |        |
| N <sub>2</sub>                               | 1.8175  | 1.4679  | 1.0480  |         |         |        |
| Al <sub>2</sub> O                            | 0.0116  | 0.0001  | 0.0000  |         |         |        |
| AlO                                          | 0.0009  | 0.0003  | 0.0000  |         |         |        |
| OH                                           | 0.0034  | 0.0574  | 0.1794  |         |         |        |
| H <sub>2</sub>                               | 2.0515  | 1.1565  | 0.1883  |         |         |        |
| HCl                                          | 0.1810  | 0.2748  | 0.3751  |         |         |        |
| H <sub>2</sub> O                             | 0.0785  | 0.8202  | 1.6139  |         |         |        |
| Condensed Phases                             |         |         |         |         |         |        |
| Al <sub>2</sub> O <sub>3</sub>               | 0.3465  | 0.2933  | 0.2096  |         |         |        |

Table V shows calculated performance data for an illustrative ratio of reactants in the propellant system Al — N<sub>2</sub>H<sub>5</sub>N<sub>3</sub> · N<sub>2</sub>H<sub>4</sub> — HClO<sub>4</sub> · 2H<sub>2</sub>O.

TABLE V

| Ingredients:                                                                 | moles   | g/100g  |
|------------------------------------------------------------------------------|---------|---------|
| Al                                                                           | 1       | 30.462  |
| N <sub>2</sub> H <sub>5</sub> N <sub>3</sub> · N <sub>2</sub> H <sub>4</sub> | 0.25    | 30.239  |
| HClO <sub>4</sub> · 2H <sub>2</sub> O                                        | 0.255   | 39.299  |
| Computed Density, lb/in. <sup>3</sup>                                        | 0.06119 |         |
| Computed Density, g/cc                                                       | 1.6935  |         |
| Performance: Frozen I <sub>p</sub> , sec                                     | 263.9   |         |
| Thermodynamic Characteristics:                                               |         | Chamber |
| Temperature, °K                                                              | 3721    |         |
| Moles of Gas, moles/100g                                                     | 3.3537  |         |
| Combustion Products, moles/100g                                              |         |         |
| Gaseous Atoms                                                                |         |         |
| Al                                                                           | 0.0311  |         |
| Cl                                                                           | 0.0285  |         |
| O                                                                            | 0.0013  |         |

|        |                                |        |
|--------|--------------------------------|--------|
| 3579   | H                              | 0.2635 |
| 3.9223 | Gaseous Molecules              |        |
|        | Al <sub>2</sub> O              | 0.0379 |
|        | AlO                            | 0.0062 |
|        | OH                             | 0.0186 |
|        | H <sub>2</sub>                 | 1.5797 |
|        | HCl                            | 0.2594 |
|        | H <sub>2</sub> O               | 0.1395 |
|        | N <sub>2</sub>                 | 0.9879 |
|        | Condensed Phases               |        |
|        | Al <sub>2</sub> O <sub>3</sub> | 0.5080 |

Table VI shows calculated performance data for an illustrative ratio of reactants in the propellant system ZrH<sub>2</sub> — LiClO<sub>4</sub> — HClO<sub>4</sub> · 2H<sub>2</sub>O.

TABLE VI

| Ingredients:                             | moles   | g/100g  |
|------------------------------------------|---------|---------|
| ZrH <sub>2</sub>                         | 1       | 66.557  |
| LiClO <sub>4</sub>                       | 0.08763 | 6.656   |
| HClO <sub>4</sub> · 2H <sub>2</sub> O    | 0.2749  | 26.787  |
| Computed Density, lb/in. <sup>3</sup>    |         | 0.1193  |
| Computed Density, g/cc                   |         | 3.3015  |
| Performance:                             |         |         |
| Shifting I <sub>p</sub> , sec            |         | 190     |
| Shifting Volumetric                      |         |         |
| I <sub>p</sub> , lb-sec/in. <sup>3</sup> |         | 22.667  |
| Frozen I <sub>p</sub> , sec              |         | 190     |
| Thermodynamic Characteristics:           |         |         |
|                                          | Chamber | Exhaust |
| Temperature, °K                          | 4073    | 2960    |
| Moles of Gas, mole/100g                  | 1.5228  | 1.4715  |
| Combustion Products, moles/100g          |         |         |
| Gaseous Atoms                            |         |         |
| H                                        | 0.2653  | 0.1714  |
| Li                                       | 0.0093  | 0.0190  |
| Cl                                       | 0.0293  | 0.0207  |
| Gaseous Molecules                        |         |         |
| H <sub>2</sub>                           | 0.9675  | 1.0140  |
| HCl                                      | 0.1346  | 0.1779  |
| LiCl                                     | 0.0533  | 0.0435  |
| ZrCl <sub>2</sub>                        | 0.0208  | 0.0083  |
| H <sub>2</sub> O                         | 0.0331  | 0.0152  |
| OH                                       | 0.0078  | 0.0013  |
| ZrO <sub>2</sub>                         | 0.0008  | 0.0000  |
| Condensed Phases                         |         |         |
| ZrO <sub>2</sub> (1)                     | 0.6921  | 0.4945  |
| ZrO <sub>2</sub> (c)                     | 0.0000  | 0.2110  |

Dihydrated perchloric acid is an intrinsically stable, only slightly toxic and caustic, oxidizer containing 73.6 percent perchloric acid and 26.4 percent water. The oxidizer is a water-white liquid with a density of 1.713 g/cc at 25° C, boiling at about 200° C and freezing at -20° C. The dihydrated acid is not even slightly caustic when cold which makes it safe for personnel and it does not require special equipment for handling.

When a lower freezing point is required for the liquid oxidizer water and/or nitric acid may be added. Both water and/or nitric acid lower the freezing point of the perchloric acid dihydrate. Water, however, lowers both the density and impulse of the oxidizer while nitric acid alone will lower the density. On the other hand, if high impulse is required and high density is of lesser importance, a higher proportion of nitric acid may be used. The addition of both water and nitric acid to the perchloric acid dihydrate makes it possible to provide oxidizer compositions having selected combinations of density, impulse and freezing point to meet a variety of requirements. The nitric acid content may be as high as 15 percent but in general compositions containing not more than about 10 percent of nitric acid are preferable as they are not unduly corrosive and are safer to handle.

The liquid oxidizer compositions of the invention consist essentially of from about 59 percent to about 77 percent by weight of perchloric acid, from 0 to about 15 percent by weight of  $\text{HNO}_3$  and the remainder water, the amount of water being sufficient to form dihydrated perchloric acid with at least about 95 percent of the perchloric acid content.

The following compositions have provided very satisfactory results:

1. 93 percent dihydrated perchloric acid (DHPA), 6 percent nitric acid and 1 percent water.
2. 90 percent DHPA, 8 percent  $\text{HNO}_3$  and 2 percent  $\text{H}_2\text{O}$ .
3. 84.2 percent DHPA, 10.5 percent  $\text{HNO}_3$  and 5.3 percent  $\text{H}_2\text{O}$ .

Table VII shows densities of selected dihydrated perchloric acid-water-nitric acid compositions.

TABLE VII

| Formulation, % by wt. |                |                      | Density, g/cc   |
|-----------------------|----------------|----------------------|-----------------|
| DHPA                  | $\text{HNO}_3$ | $\text{H}_2\text{O}$ | Measured        |
| 86.8                  | 8.0            | 5.2                  | 1.58 $\pm$ 0.03 |
| 78.5                  | 16.5           | 5.0                  | 1.54 $\pm$ 0.03 |
| 90                    | 9.0            | 2.0                  | 1.67 $\pm$ 0.03 |

The improved oxidizers of the invention may be advantageously employed with a wide variety of light metals, metal hydrides, mixtures of light metals and metal hydrides, and light metals and metal hydrides admixed or combined with other compatible fuels. The following list is exemplary of suitable fuels which may be employed with the oxidizers of the invention: Zr; Al;  $\text{AlH}_3$ ;  $\text{ZrH}_2$ ; Mg;  $\text{Mg}(\text{AlH}_4)_2$ ;  $(\text{AlH}_3)_2\text{NH}_3$ ;  $(\text{AlH}_3)_2\text{N}_2\text{H}_4$ ;  $\text{TiH}_2$ ; and  $\text{MgH}_2$ . Of these fuels Zr,  $\text{ZrH}_2$ , and  $\text{AlH}_3$  have been found to be particularly suitable for rocket fuels with the oxidizers of the invention.

We claim:

1. A method of producing thrust which comprises reacting in a combustion chamber an oxidizer comprising substantially dihydrated perchloric acid and a fuel selected from the group consisting of light metals, metal hydrides and mixtures thereof.
2. A method of producing thrust which comprises reacting in a combustion chamber an oxidizer comprising substantially dihydrated perchloric acid and a fuel consisting predominantly of a light metal.
3. A method of producing thrust which comprises reacting in a combustion chamber an oxidizer comprising substantially dihydrated perchloric acid and a fuel consisting predominantly of a metal hydride.
4. A method of producing thrust which comprises reacting in a combustion chamber an oxidizer comprising

ing substantially dihydrated perchloric acid and a fuel consisting predominantly of Zr.

5. A method of producing thrust which comprises reacting in a combustion chamber an oxidizer comprising substantially dihydrated perchloric acid and a fuel consisting predominantly of  $\text{ZrH}_2$ .

6. A method of producing thrust which comprises reacting in a combustion chamber an oxidizer comprising substantially dihydrated perchloric acid and a fuel consisting predominantly of  $\text{AlH}_3$ .

7. A method of producing thrust which comprises reacting in a combustion chamber an oxidizer comprising a liquid composition consisting essentially of from about 59 percent to about 77 percent by weight of perchloric acid, from 0 to about 15 percent by weight of  $\text{HNO}_3$  and the remainder water, the amount of water being sufficient to form dihydrated perchloric acid with at least about 95 percent of the perchloric acid and a fuel selected from the group consisting of light metals, metal hydrides, and mixtures thereof.

8. A method of producing thrust which comprises reacting in a combustion chamber an oxidizer comprising about 90 percent by weight of dihydrated perchloric acid, about 8 percent by weight of nitric acid and about 2% by weight of water and a fuel selected from the group consisting of light metals, metal hydrides, and mixtures thereof.

9. A method of producing thrust which comprises reacting in a combustion chamber an oxidizer comprising about 84.2 percent by weight of dihydrated perchloric acid, about 10.5% by weight of nitric acid and about 5.3 percent by weight of water and a fuel selected from the group consisting of light metals, metal hydrides, and mixtures thereof.

10. In a rocket propellant system a liquid oxidizer consisting essentially of from about 59 percent to about 77 percent by weight of perchloric acid, from 0 to about 15 percent by weight of  $\text{HNO}_3$  and the remainder water, the amount of water being sufficient to form dihydrated perchloric acid with at least about 95 percent of the perchloric acid.

11. In a rocket propellant system a liquid oxidizer consisting essentially of about 90 percent by weight dihydrated perchloric acid, about 8 percent by weight nitric acid and about 2 percent by weight water.

12. In a rocket propellant system a liquid oxidizer consisting essentially of about 84.2 percent by weight dihydrated perchloric acid, about 10.5 percent by weight nitric acid and about 1 percent by weight water.

13. In a rocket propellant system a liquid oxidizer consisting essentially of about 84.2 percent by weight dihydrated perchloric acid, about 10.5 percent by weight nitric acid, and about 5.3 percent by weight water.

\* \* \* \* \*